

## UNITED STATES PATENT OFFICE

2,110,394

LEATHER DYED WITH MONO- OR DISAZO  
DYESTUFFS

Ernst Fellmer, Leverkusen-I. G. Werk, Gustav Mauthe, Cologne-Holweide, and Hermann Noerr, Leverkusen-I. G. Werk, Germany, assignors to General Aniline Works, Inc., New York, N. Y., a corporation of Delaware

No Drawing. Application March 18, 1936, Serial No. 69,592. In Germany March 23, 1935

4 Claims. (Cl. 8—5)

The present invention relates to leather dyed with certain mono- or disazodyestuffs, more particularly it relates to leather which has been dyed with mono- or disazodyestuffs of the general formula:



In the said formula R stands for the radical of an aromatic diazo compound or a diazo compound derived from a monamine or monamines respectively, R' stands for a 2-aminonaphthol-coupling component or a substitution product thereof, especially of such a substitution product in which a hydrogen atom of the amino group is substituted by alkyl or aryl or substituted alkyl or aryl, e. g. the sulfo or carboxylic acids thereof, and n stands for a whole number, such as for 1, 2, 3 or 4 etc.

In dyeing chrome leather, it is desired not only to dye the surface of the leather, but also to give an even shade to the cut of the leather to a certain depth of penetration, while the zone of the cross-cut remaining undyed is intended to retain the pure greenish chrome color.

Of particular technical importance are dyeings of this kind on leathers, the grain side or flesh side of which is more or less ground off after the dyeing.

In accordance with the present invention the desired effect is attained to an excellent degree, when in the dyeing process mono- or disazodyestuffs of the above identified formula are used, the dyeing per se being performed according to the standard methods of dyeing leather, as is more fully described in the annexed examples. If desired the mono- or disazodyestuffs of the above identified formula can be used in mixture with other acid or substantive dyestuffs.

The invention is illustrated by the following examples, without being restricted thereto:

Example 1.—100 kgs. of neutralized chrome calf leather are introduced into a drum with about 300 kgs. of water at 60° C. A dyestuff solution is gradually added prepared from 1 kg. of the dyestuff from diazotized p-sulfanilic acid coupled with phenyl gamma acid (alkaline coupling) and 25 kgs. of hot water. After half an

hour, the dyestuff has been absorbed almost without residue. Stuffing of the leather is then effected. In this manner, there is obtained a dyeing of a useful brown shade, which exhibits on the grain side and on the flesh side a distinct dyeing of the cut, without change of the characteristic greenish color of the chrome leather in the interior of the cut. After glacé finishing such leathers exhibit an improvement of covering and equalizing properties in comparison with leathers dyed with dyestuffs which do not dye in the grain in the manner described. Further, the flesh side can be easily ground off, an operation which is usual in many cases, without producing a bad and ununiform appearance by the standing out of undyed fibers.

Example 2.—100 kgs. of dry and ground off chrome calf velours leather are dyed, after a good egging in 500 kgs. of hot water, with 5 kgs. of the dyestuff obtained from diazotized sulfanilic acid coupled in an alkaline medium with 1 molecular proportion of a mixture of 60% phenyl-gamma-acid and 40% phenyl-J-acid. In order entirely to exhaust the dye bath, it is acidified with formic acid, and finally, as usual for velours leather, the latter is subjected to some degree of stuffing.

There are obtained dyeings of a reddish brown shade, which exhibit a very strong dyeing in the grain. The leathers dyed in this manner show a good fastness to grinding off and to water, and there is not the lightening of shade, which in other cases is a troublesome result of re-grinding.

Example 3.—100 kgs. of chrome tanned and neutralized horse leather are dyed in a bath with 0.75 kgs. of the dyestuff from diazotized 4-nitraniline-2-sulfonic acid coupled with phenyl-gamma-acid (acid coupling) with the addition to the bath of 0.75 kgs. of direct deep black E extra (Schultz Farbstofftabellen 1931, p. 271), and then stuffed. The leather dyed in this manner gives a black shade with a deep dyeing in the grain, so that it is possible to grind off the grain, as is usual in the manufacture of horse leather, without rendering visible undyed interior zones.

The following table contains some further examples and the shades obtained on leather:

| Diazo components                       | Coupling components                                       | Shade           |
|----------------------------------------|-----------------------------------------------------------|-----------------|
| 5 0-Sulphanilic acid                   | Phenyl gamma acid (alkaline coupling)                     | Brown           |
| Do                                     | Phenyl-J-acid (alkaline coupling)                         | Red             |
| 10 2-naphthylamine-4,8-disulfonic acid | Phenyl gamma acid (alkaline coupling)                     | Brown           |
| Aniline                                | m-Carboxyphenyl gamma acid (alkaline coupling)            | Reddish brown   |
| Amino-azobenzene                       | 2,8-aminonaphthol-3,6-disulfonic acid (alkaline coupling) | Violet brown    |
| 15 4-nitraniline-2-sulfonic acid       | Phenyl gamma acid (acid coupling)                         | Bluish grey     |
| 15 5-nitro-2-anisidine-4-sulfonic acid | Phenyl gamma acid (acid coupling)                         | Violetish grey  |
| Do                                     | Phenyl-J-acid (acid coupling)                             | Bordeaux        |
| 20 2-nitraniline-4-sulfonic acid       | 2,3-aminonaphthol-6-sulfonic acid (acid coupling)         | Yellowish brown |
| Metanilic acid                         | 2,3-aminonaphthol-6-sulfonic acid (acid coupling)         | Yellowish brown |
| 20 Sulfanilic acid                     | 2-(o-hydroxyethylamino)-8-naphthol-6-sulfonic acid        | Brown           |
| Aminoazobenzene disulfonic acid        | Gamma acid (acid coupling)                                | Violet          |
| Do                                     | Phenyl gamma acid (alkaline coupling)                     | Dark brown      |
| 25                                     |                                                           |                 |

Besides the excellent dyeing obtained in a neutral bath, the dyestuffs have a good stability to alkalies and acids and in general also a good fastness to alkalies and acids.

30 The dyestuffs in question, besides being suitable for chrome leather, are particularly suitable for dyeing other kinds of leather, especially vegetable and semichrome tanned leather. Of course, they can also be used together with other suitable acid or substantive dyestuffs.

We claim:

1. Leather dyed with a dyestuff of the general formula:



in which R stands for a member selected from the group consisting of radicals of diazo and diazoazo compounds derived from monamines, R' stands for a member selected from the group consisting of radicals of 2-aminonaphthol-coupling components and of N-substitution products thereof, and n stands for a whole number.

2. Leather dyed with a dyestuff of the general formula:



in which R stands for the radical of a diazotized monamine of the benzene series and R' for the radical of a 2-aminonaphthol-coupling component in which one hydrogen atom of the amino group is substituted by aryl, and n stands for a whole number.

3. Leather dyed with the dyestuff having in the free state the following formula:



4. Leather dyed with the dyestuff having in the free state the following formula:



ERNST FELLNER,  
GUSTAV MAUTHE,  
HERMANN NOERR.

40

50

60